

## UNITED STATES PATENT OFFICE.

WALther DUISBERG, OF LEVERKUSEN, NEAR COLOGNE, AND WINFRID HENTRICH AND LUDWIG ZEH, OF WIESDORF, NEAR COLOGNE, GERMANY, ASSIGNS TO GRASSELLI DYESTUFF CORPORATION, OF NEW YORK, N. Y., A CORPORATION OF DELAWARE.

## PROCESS OF DYEING CELLULOSE COMPOUNDS.

No Drawing. Application filed March 18, 1925, Serial No. 16,567, and in Germany March 18, 1924.

We have invented new and useful improvements in the dyeing of cellulose compounds such as cellulose esters or ethers and in the products so obtained.

5 Our invention relates to the use of anthraquinone derivatives which have affinity for cellulose compounds such as cellulose acetate, cellulose formate, ethyl cellulose, propyl cellulose or other organic cellulose esters and cellulose ethers. Especially suitable are 10 water soluble anthraquinone derivatives, for example, alkaline earth metal salts such as the sodium salts. For the purpose of this invention we will call these cellulose derivatives organo-oxy-cellulose compounds.

15 We have now found that amino-anthraquinone-N-methyl- $\omega$ -sulfonic acid compounds are easily absorbed by organo-oxy-cellulose compounds and that shades ranging practically over the whole color scale can be obtained by dyeing organic cellulose esters and cellulose ethers in aqueous solution with such products. This process is exceedingly valuable for obtaining fast and brilliant shades 20 on textile products made out of such cellulose compounds and in so-called mixed goods it allows to obtain various effects especially when the other textile fibres woven together with the cellulose ester or cellulose ethers have a different affinity for these anthraquinone dyes.

25 The amino-anthraquinone-N-methyl- $\omega$ -sulfonic acid compounds referred to are of the general type



30 They are obtained by treating the corresponding amino anthraquinones with formaldehyde and an alkali metal bisulfite in aqueous and eventually acid suspension.

35 Other substitution in the anthraquinone nucleus as for instance by hydroxyl groups though modifying the shade, will not influence the dyeing properties for organo-oxy-cellulose compounds.

40 Our invention will be further illustrated by the following examples, the parts being by weight:

45 Example 1.—Six parts of the sodium salt

of 1-4-diamino-anthraquinone-N-methyl- $\omega$ -sulfonic acid



55

are dissolved in 10,000 parts hot water. 250 parts cellulose acetate silk are entered into this dye bath at about 70° C. and treated for 3/4 of an hour at this temperature. After wringing, washing and drying, the silk is 60 dyed a clear bright violet. 65

Example 2.—Six parts of the sodium salt of 1-5-dihydroxy-4-8-diamino-anthraquinone-N-methyl- $\omega$ -sulfonic acid



70

75

are dissolved in 10,000 parts of water and 300 parts ethyl cellulose threads dyed for 3/4 of an hour at 70° C. in this bath. Clear, 80 bright, blue shades are obtained.

Example 3.—Six parts of the sodium salt of 1-4-5-8-tetra-amino-anthraquinone-N-methyl- $\omega$ -sulfonic acid



85

90

are dissolved in 10,000 parts of water. 250 parts cellulose formate silk are dyed in this bath at about 70° C. for 3/4 of an hour. A 95 deep, bright greenish-blue shade is obtained.

In the same way beta-aminoanthraquinone-N-methyl- $\omega$ -sulfonic acid compounds can be used.

We claim:

1. The process of dyeing organo-oxy-cellu-

100

lose compounds which consists in treating same with amino-anthraquinone-N-methyl- $\omega$ -sulfonic acid compounds.

2. The process of dyeing organo-oxy-cellulose compounds which consists in treating same with aqueous solutions of soluble amino-anthraquinone - N - methyl- $\omega$ -sulfonic acid compounds.

3. The process of dyeing cellulose acetate 10 which consists in treating same with amino-anthraquinone - N - methyl- $\omega$ -sulfonic acid compounds.

4. The process of dyeing cellulose acetate which consists in treating same with aqueous 15 solutions of soluble amino-anthraquinone-N-methyl- $\omega$ -sulfonic acid compounds.

5. The process of dyeing organo-oxy-cellulose compounds which consists in treating same with 1-4-diamino-anthraquinone-N- 20 methyl- $\omega$ -sulfonic acid compounds.

6. The process of dyeing organo-oxy-cellulose compounds which consists in treating same with aqueous solutions of soluble salts of 1-4-diamino-anthraquinone-N-methyl- $\omega$ - 25 sulfonic acids.

7. The process of dyeing cellulose acetate

which consists in treating same with 1-4-diamino-anthraquinone-N-methyl- $\omega$ -sulfonic acid compounds.

8. The process of dyeing cellulose acetate 30 which consists in treating same with aqueous solutions of soluble salts of 1-4-diamino-anthraquinone-N-methyl- $\omega$ -sulfonic acids.

9. As new products organo-oxy-cellulose compounds dyed with amino-anthraquinone- 35 N-methyl- $\omega$ -sulfonic acid compounds.

10. As new products organo-oxy-cellulose compounds dyed with soluble salts of 1-4-diamino-anthraquinone-N-methyl- $\omega$ -sulfonic acids. 40

11. As new products cellulose acetate compounds dyed with soluble salts of 1-4-diamino-anthraquinone-N-methyl- $\omega$ -sulfonic acids.

12. As new products cellulose acetate compounds dyed with amino-anthraquinone-N-methyl- $\omega$ -sulfonic acid compounds. 45

In testimony whereof we have hereunto set our hands.

WALTHER DUISBERG.  
WINFRID HENTRICH.  
LUDWIG ZEH.